

## UNITED STATES PATENT OFFICE.

WALTER F. GRAHAM, OF BALTIMORE, MARYLAND, ASSIGNOR, BY MESNE ASSIGNMENTS, TO U. S. INDUSTRIAL ALCOHOL CO., A CORPORATION OF WEST VIRGINIA.

## NICKEL-COPPER ALLOY.

No Drawing.

Application filed August 28, 1923. Serial No. 659,837.

*To all whom it may concern:*

Be it known that I, WALTER F. GRAHAM, a citizen of the United States, a resident of Baltimore and State of Maryland, have invented a certain new and useful Nickel-Copper Alloy, of which the following is a specification.

This invention relates to nickel copper alloys having a comparatively low percentage of nickel with respect to Monel metal or similar alloys but having at the same time the desirable characteristics of high nickel alloys.

The invention has as an object the production of nickel copper alloys containing iron in small amounts for use in manufacturing forge materials and for other purposes. It is an object of the invention to eliminate soft metals such as lead and zinc in order to avoid the uneven texture and hardness and the difficulty of working due to large amounts of such soft metals. A further object is to produce a white metal of decreased nickel content at minimum expense without incurring the losses hitherto experienced in the prior practice of making white metals of this character. Further objects of the invention will appear hereinafter.

By way of a preferred embodiment two specific examples will be given, which are as follows:

A mix is made of nickel 30 to 35%, iron 5 to 7%, a deoxidizer such as silicon, manganese, or zirconium about 1% or less, and the balance copper. This mix is particularly advantageous for making superheat metals for use in steam fittings, valves, pipes, etc.

Another composition consists of nickel 35%, iron 3 to 5%, and the remainder copper, together with a deoxidizer as in the foregoing example.

These mixes when melted in any suitable way will produce alloys having high resistance qualities against corrosion, high tensile

strength, uniformity, even texture, and they will be comparatively easy to melt. The casting may if desired be performed by a special process in a mold wherein the temperature gradient is controlled, such as an iron mold dusted with graphite. When casting in this manner the rapid drop in temperature will freeze out a maximum concentration of the nickel rich constituent, whereby there will be obtained the same desirable qualities possessed by high nickel alloys, such as Monel metal, without incurring the disadvantages attendant upon fusing high nickel mixes. The nickel may, if desired, range up to 45% but not over 50%, although it is desirable to keep it within the ranges named in the above preferred embodiments. Instead of using Monel metal for the mix, as is customary in this art, it is preferred to use pure metals, thereby avoiding the impurities and small amounts of other metals contained in Monel metal.

As many apparently widely different embodiments of my invention may be made without departing from the spirit thereof, it is to be understood that I do not limit myself to the embodiments described except as defined in the following claims.

I claim:

1. An alloy consisting of nickel 30 to 35%, iron 3 to 7%, and the remainder copper, and containing no lead or zinc.
2. A ternary copper alloy containing from 30 to 40% nickel and from 3 to 7% iron.
3. A ternary copper alloy containing from 30 to 40% nickel and about 5% iron.
4. A ternary copper alloy containing from 30 to 45% nickel, from 3 to 7% iron, and containing no lead or zinc.

In testimony that I claim the foregoing, I have hereunto set my hand this 18th day of August, 1923.

WALTER F. GRAHAM.